

## UNITED STATES PATENT OFFICE

2,193,011

## COLORED PHOTOGRAPHIC IMAGE

Karl Schinzel, Rochester, N. Y., assignor to Eastman Kodak Company, Rochester, N. Y., a corporation of New Jersey

No Drawing. Application December 30, 1938,  
Serial No. 248,517. In Austria May 9, 1936

5 Claims. (Cl. 95—88)

This invention relates to color photography and particularly to a method for forming colored images in photographic layers.

This application is a continuation in part of my prior application, Serial No. 139,759, filed April 29, 1937.

Modern processes of color photography involve the formation of three-color separation images in a photographic film. The formation of colored images in this way is usually accomplished by sensitizing a single photographic layer to three regions of the visible spectrum or by coating three differentially sensitized layers on the same side or on opposite sides of a photographic support. In processes of this type it is frequently difficult to form the third color image without affecting the two previously formed images or to form a colored image in the middle layer of three layers coated on the same side of a single support.

It is, therefore, the principal object of the present invention to provide a method for forming a colored image in a photographic layer by a chemical method which does not affect previously formed images. A further object is to provide a method for forming a colored photographic image by direct chemical conversion. Other objects will appear from the following description of my invention.

These objects are accomplished according to my invention by the direct conversion of a silver salt such as silver halide or silver ferrocyanide into a colored photographic image.

In processes of color photography, such as those described in my prior application, Serial No. 139,759, three differentially sensitized layers may be coated on the same side of a single photographic support. After exposure of a film of this nature it is necessary to form three differently colored images in the separate layers. For example, where the layers are sensitive, respectively, to the red, green, and blue regions of the spectrum, the final images are colored, respectively, blue-green, magenta and yellow. Dye images may be formed in various ways in these layers as by toning, color coupling, etc. The image in the layer nearest the support is usually colored first and the image in the middle layer or top layer colored second. The final image must be colored by some means which does not destroy or adversely affect the images in the other layers. This is frequently a difficult procedure particularly in a reversal process where there is a sensitive silver salt in the layers after the primary development.

I have found that after the formation of a colored image in one of the layers of a multi-layer film, for example, in the layer nearest the support, and in one of the remaining layers, that an image in the third layer may be formed by a direct conversion of the remaining silver salt into colored substances or into mordants or basic dyes or into precipitants or acid dyes. This last method is not preferred since acid dyes usually stain the gelatin and cannot be washed out of the highlight portions as easily as basic dyes. The sensitive silver salt, for example, silver chloride or silver bromide may be treated directly or may be converted into ferrocyanide and treated as silver ferrocyanide. It is more desirable first to remove any metallic silver remaining after the formation of the first two part-color images, to reduce the silver halide of the remaining emulsion to metallic silver and to convert it into silver ferrocyanide or a mixture of silver ferrocyanide with lead ferrocyanide by means of potassium ferricyanide.

This procedure can be followed for the formation of an image in the middle emulsion layer or in the top emulsion layer. The silver salt in the top emulsion layer might be converted to a color compound according to the present process before the formation of an image in the middle, or both the middle or lower emulsion layers if the colored compound formed from the silver halide is one which resists the development. According to the preferred method of carrying out my invention, however, the silver halide is converted to the colored compound according to the present process only after colored images are formed in the other two emulsion layers.

The method for forming the colored image from silver halide according to my invention involves the chemical conversion of the silver salt into a colored compound upon treatment with certain compounds containing the mercaptan group. The compound formed in this way is a silver salt which is much less soluble than the original silver halide, and the conversion is performed chemically, not depending on exposure of the silver salt to form a latent image. Compounds, such as thio-glycolic acid anilide and thio-glycolic- $\beta$ -naphthalide, for example, form yellow precipitates with silver salts and may be used to form yellow images in photographic layers according to my invention. The ferrocyanides of silver and other metals are also suited for conversion into colored compounds with mercaptans to form yellow or red salts. All of these reactions can, of course, be accomplished with the

residual silver chloride of reversal development as well as with the silver chloride or ferrocyanide of the middle layer in three-color redevelopment.

Other thioglycolic acid derivatives that can be used according to my invention include the following compounds:



(where  $\mathbf{X}$  is



45 It is frequently desirable to add a small amount of a silver halide solvent to the solution in order to increase the solubility of the silver halide so that it reacts with the mercaptan more easily. For example, 2 or 3% of thiourea in a solution 50 of the mercaptans or their alkali metal or ammonium salts aids in the conversion of the silver halide into a colored compound.

The mercaptans used in the treatment of the silver salt image may be formed in various ways 55 which appear more simple to substitute the sulfhydryl group in aromatic amines or vat dyes which contain a diazotizable amino group by means of xanthogenate and subsequent saponification. Anthraquinone or vat dyes with thiophenol groups or intermediate products can also be used directly for this purpose. The introduction of the thioglycolic acid residue into the amino compounds mentioned or also into those 60 with hydroxyl or sulfhydryl groups is most easily accomplished by first forming the chloracetyl derivative, if necessary in the presence of tertiary aromatic bases and then condensing two molecules of this compound with sodium disulfide 65 or polysulfide to the organic disulfide which

yields the mercaptan by reduction. The carboxylic acid chlorides or sulfonic acid chlorides of dyes such as thioindigo can be reacted with phenol, ortho or para disulfide or with dithio-m-toluylene diamine and then reduced to the mercaptan by mild reducing agents. The disulfide of the mercapto aldehyde can be condensed to anils with the amino group of the initial substances mentioned above and then reduced. Aromatic disulfides of sulfochlorides can also be 10 used for forming a chain of the initial substance or of amino dyes and then decomposed by reduction to the mercaptan derivative. This reaction can also be used to form the mercaptide of quinoline yellow, dithioanthrarufine, thiazols, 15 oxazines and the synthetic sulfur dyes. In many cases, the sulfochlorides of the initial substances and dyes can easily be reduced to the corresponding mercaptans.

It is to be understood that colored photographic images according to my invention can be formed in any of the layers of a multi-layer film or in a single layer sensitive to only the spectral region or containing differentially sensitized silver halide grains. Mercaptans other 20 than those specifically mentioned can be used and numerous other modifications may be made in the various aspects of my invention. It is to be understood that my invention is to be limited only by the scope of the appended claims.

Having thus described my invention, what I claim as new and desire to be secured by Letters Patent is:

1. The method of forming a colored photographic image in a silver halide layer containing 35 a silver salt image which comprises treating said layer with a solution of a thioglycolic amide containing a group selected from the class consisting of aromatic and heterocyclic groups.

2. The method of forming a colored photographic image in a gelatin layer containing a silver halide image which comprises treating said layer with a solution of a thioglycolic amide containing a group selected from the class consisting of aromatic and heterocyclic groups to 45 convert the silver halide into a colored silver salt.

3. The method of forming a colored photographic image in a gelatin layer containing a silver bromide image which comprises treating 50 said layer with a solution of a thioglycolic amide containing a group selected from the class consisting of aromatic and heterocyclic groups to convert the silver bromide into a colored silver salt.

4. The method of forming a colored photographic image in a gelatin layer containing a silver halide image, which comprises treating 55 said layer with a solution of thioglycolic- $\beta$ -naphthalide to form a yellow silver salt image 60 in the layer.

5. The method of forming a colored photographic image in a gelatin layer containing a silver halide image, which comprises treating the 65 layer with a solution of a thioglycolic amide containing a group selected from the class consisting of aromatic and heterocyclic groups, and a silver halide solvent, to form a colored silver salt image in the layer.